

Jan. 21, 1941.

A. J. LANGHAMMER ET AL

2,229,330

POROUS METAL PRODUCT AND METHOD OF MAKING SAME

Filed March 8, 1937



Fig. 2.



Fig. 1.



Fig. 5.



Fig. 3.



Fig. 4.

INVENTOR  
ANTHONY J. LANGHAMMER AND  
BY WILLIAM G. CALKINS.  
Hansen Lind Paten & Hanis  
ATTORNEYS

## UNITED STATES PATENT OFFICE

2,229,330

POROUS METAL PRODUCT AND METHOD OF  
MAKING SAME

Anthony J. Langhammer and William G. Calkins,  
Detroit, Mich., assignors to Chrysler Corporation,  
Highland Park, Mich., a corporation of  
Delaware

Application March 8, 1937, Serial No. 129,595

2 Claims. (Cl. 75—22)

This invention relates to improvements in compressed and sintered powdered metal articles and in the method of making the same.

More specifically, the invention pertains to improved metal articles of this character which are of a porous nature and particularly useful in friction and anti-friction elements, such as bearings.

One of the main objects of the invention is to improve the physical characteristics, such as ductility and strength of powdered metal products of this kind, by increasing the adhesion of the powdered metal particles to each other, and particularly by increasing the number of individual bonds between adjacent particles of powdered metal.

Another object of the invention is the provision of articles fabricated from a mixture of powdered metals having different melting points, in which the quantity of powdered metal of higher melting point by far exceeds the quantity of powdered metal of lower melting point, but in which there are present substantially as many or more particles of the powdered metal of lower melting point.

Further objects of the invention are to provide articles of this character in which there are present at least one particle of the powdered metal of lower melting point to bond each particle of powdered metal of higher melting point to the next adjacent similar particle; to provide a mixture of such powdered metals in which the particles of lower melting point are substantially smaller than those of higher melting point; and to provide a compressed and sintered powdered metal structure which has substantially each particle of metal of higher melting point bonded to each adjacent particle of similar metal by a particle of the metal of lower melting point.

An illustrative embodiment and diagrammatic explanation of the invention is shown in the accompanying drawing, in which:

Fig. 1 is a diagrammatic illustration of the approximate relationship and comparative size of particles of powdered metal included in powdered metal mixtures used in manufacturing articles embodying the invention.

Fig. 2 is a diagrammatic illustration of the approximate relationship and relative size of the articles of powdered metal conventionally used in the manufacture of compressed and sintered bearing products.

Fig. 3 is a sketch of a micro-photograph of the powdered metal of lower melting point, used in manufacturing porous bearing articles embody-

ing the invention and magnified approximately 172 times, the particular metal photographed being copper.

Fig. 4 is a sketch of a micro-photograph of the powdered metal of higher melting point, used in manufacturing porous metal articles embodying the invention and magnified approximately 172 times, the particular metal photograph being of powdered sponge iron.

Fig. 5 is a perspective view of a bearing embodying the invention.

Powdered metal products of the type to which this invention relates may be put to numerous uses, but because of the porosity and lubricant absorbing capacity of such products, they are particularly suitable for bearing purposes. In general, products of this kind are manufactured by thoroughly mixing together two or more powdered metals in selected proportions. The powdered metals usually have different melting points, and there is present a substantially greater quantity of the powdered metal of higher melting point than that of the lower melting point. In addition to the powdered metals, which constitute the main constituents of the mixture, there may be added relatively small quantities of solid lubricants such as graphite, which it may be desired to retain in the final product. The mixture may also contain volatile or other lubricants which are mainly removed during the sintering operation, these materials being provided to lubricate the surfaces of the dies or molds in which the powdered mixture is compressed.

The powdered constituents of the mixture are thoroughly incorporated together and distributed throughout each other by a suitable mixing operation and they are then compressed under high unit pressure into briquettes of desired shape. The briquettes are then removed from the die and sintered, preferably in a reducing or non-oxidizing atmosphere, at a temperature above the melting point of the powdered metal of lower melting temperature and below the melting temperature of the metal of higher melting point. During this sintering operation, the particles of metal of higher melting point are bonded together by the particles of metal of lower melting point.

For the purpose of illustration, powdered iron and powdered copper particles are shown in the drawing, although combinations of other metals of different melting points may be used to equal advantage in the practice of the invention.

In Fig. 1 of the drawing, there is diagrammatically illustrated the relationship and relative

size of one unit of a mixture of powdered iron and copper suitable for the formation of compressed and sintered porous bearing products. In the illustration shown, there are nine large circles 10, which represent particles of powdered iron, and ten small circles 11, which represent particles of powdered copper. Each particle of powdered iron is shown to be approximately of the order of ten times as large as a corresponding 10 particle of powdered copper 11, this illustration being diagrammatically illustrative of the relative average sizes of a large number of particles. This figure approximately represents the relative size of the particles of iron and copper in a mixture comprising substantially ten percent copper and ninety percent iron, the size of the particles being illustrative of the quantity by weight thereof.

By thoroughly mixing the powdered metal, an arrangement thereof corresponding approximately 20 to the diagrammatic illustration shown in Fig. 1 is obtainable. Each particle of iron 10 has between it and the next successive particle of iron a small particle of copper 11 and by predetermining the sizes of the particles such that there is a greater number of particles of copper than particles of iron, an extra particle, or extra particles of copper may be provided in a central location with respect to the particles of iron. When the 25 particles of a mixture of powdered iron and powdered copper are arranged in a manner approaching that illustrated in Fig. 1, and the mixture is then compressed and sintered, the particles of powdered copper between adjacent particles of powdered iron fuse and provide bonds between the iron particles. The centrally located particle of powdered copper also fuses to provide additional bonds between all of the particles of powdered iron with which it is associated. In this manner, each particle of powdered iron is 30 rigidly bonded to an adjacent particle of powdered iron by several copper bonds.

When the particles of powdered copper are substantially the same size as the particles of powdered iron, as illustrated in Fig. 2, or larger than the iron particles, the number of bonds between the particles of powdered iron resulting from the sintering operation is materially less than the number of bonds provided by the invention.

From a consideration of the micro-photograph shown in Figs. 3 and 4, it is obvious that a mathematically accurate and precise relationship of sizes of powdered metals of different melting temperatures and arrangement thereof, such as that shown in Fig. 1, cannot be obtained, but by properly predetermining the size of the metals of different melting points and taking into account the quantity and density thereof, it is possible to approach or approximate the arrangement and relative sizes illustrated in this figure. In general, 45 it is sufficient to obtain meritorious results from practice of the invention if the particles of metal of lower melting point are present in number of substantially the same order as the number of particles of metal of higher melting point. When this condition exists, the resulting bearing 44, shown in perspective in Fig. 5, has all of its powdered metal particles rigidly bonded together by a much larger number of bonds than have been heretofore provided and the porous structure is therefore less susceptible to fracture and capable of 50 withstanding greater loads. The increased number of bonds between the metal particle re-

sults in an increase in both structural strength and ductility of the finished product.

The powdered metals should preferably have the following screen analysis:

Iron particles

All through 150 mesh

Approximately 75% will be collected on screens of between 150 and 325 mesh

Approximately 25% through 325 mesh.

Ninety percent of the powdered copper particles should be capable of passing through a 325 mesh screen.

This invention may be practiced in the formation of porous products manufactured from mixtures of powdered materials having the following compositions:

|                     | Per cent by weight |
|---------------------|--------------------|
| Powdered copper     | 88.5               |
| Powdered tin        | 10                 |
| Powdered graphite   | 1.5                |
| Powdered copper     | 20                 |
| Powdered graphite   | 1.2                |
| Powdered boric acid | 1                  |
| Powdered iron       | 25                 |
|                     | 77.5               |

Regardless of the particular proportions and nature of the constituents of mixtures of powdered material from which porous metal products may be formed, predetermining of the size of the particles of higher melting point with respect to the particles of metal of lower melting point in accordance with this invention, will result in the attainment of superior structural properties in the final products formed from the mixture.

Although but several specific embodiments of the invention is herein shown and described, it will be understood that various changes in the size, shape and arrangement of parts may be made without departing from the spirit of our invention.

We claim:

1. A sintered porous bearing structure comprising substantially 90% by weight of powdered iron and substantially 10% by weight of powdered copper particles, the particles of powdered copper being fused to adjacent particles of powdered iron for providing a substantially fused bond therebetween and being of such order of size that when unfused substantially 90% thereof will pass through a 325 mesh screen and said particles of powdered iron being of such order of size that substantially all thereof will pass through a 150 mesh screen, substantially 75% thereof will be collected on screens of between 150 to 325 mesh and substantially 25% thereof will pass through a 325 mesh screen.

2. The method of making a porous metal bearing structure which comprises compressing into a briquette a mixture comprising substantially 10% by weight of powdered copper and 90% by weight of powdered iron, the particles of powdered iron being of an average size in volume approximately ten times that of the average size in volume of the particles of powdered copper, and sintering said briquette in a non-oxidizing atmosphere at a temperature between the melting temperature of said powdered iron and said powdered copper for forming fused bonds between portions of adjacent particles of said powdered iron.

ANTHONY J. LANGHAMMER.  
WILLIAM G. CALKINS.